

## UNITED STATES PATENT OFFICE

BORIS N. LOUGOVY, OF NEW YORK, N. Y., ASSIGNOR TO CHADELOID CHEMICAL COMPANY, OF NEW YORK, N. Y., A CORPORATION OF WEST VIRGINIA

## HEAVY-BODIED FINISH REMOVER CONTAINING A CORRECTIVE OF ANTI-PENETRATION

No Drawing.

Application filed November 30, 1928. Serial No. 322,968.

This invention relates to a finish remover especially adapted for work on vertical surfaces and particularly refers to a heavy bodied mixture containing wax and nitrocellulose and so balanced as to produce the quickest possible action when applied to a painted surface.

With a general type of remover composed of a mixture of solvents with an appropriate proportion of wax, such as, for example, removers containing mixtures of benzol and acetone with or without alcohol, to which 3 to 5% of wax has been added, there is often difficulty in working on vertical surfaces because such removers run down and consequently the remover does not stay in contact with the finish on the upper part of the surface sufficiently long to produce the desired loosening action on the paint.

It therefore has been deemed necessary to produce a type of paint and varnish remover which will stay on vertical surfaces without running down. This has usually been accomplished by increasing the body of the remover by incorporating substances capable of forming colloidal solutions such as esters of cellulose, soaps, etc. Nitrocellulose in the form of old moving picture film or celluloid scrap is the most widely used material for such purpose. An increase in the proportion of wax in conjunction with nitrocellulose also has been employed as a means to increase the body.

However, the addition of various solids which are capable of dissolving in one of the solvents present in a paint and varnish remover will result in cutting down the speed of attack of a given solvent or of a mixture of several solvents, and therefore the cutting speed or rate of attack of a remover containing such substances as wax or nitrocellulose is accordingly slower than the cutting speed of a corresponding mixture which does not contain such solids. Such substances could be termed "anti-penetrants", since they prevent or retard penetration of the remover into the finish coating.

The method adopted for measuring the activity of the paint and varnish remover solvents was as follows: A piece of old painted

wood was selected, taking care that the portion used had a good even, thick coat of paint, and this was cut into strips. The solvent mixture to be tested was placed in a test tube and a strip of the painted wood was put into this test tube. The time which elapsed before the first appearance of any wrinkling was noted accurately by means of a stop watch. The comparative "removing action" was thus roughly represented by the number of seconds, being inversely proportional to these numbers. In addition to this, each completed paint and varnish remover composition was also tested on the same kind of a painted surface and under the conditions approximating the actual use of removers in practice. For this purpose a part of an old automobile (finished with an oil paint) was secured. Each remover was placed on the surface in approximately the same quantity and the time was noted by means of a stop watch when the blistering or wrinkling of the surface was plainly observable. The cutting power was then represented by the number of seconds which elapsed before the appearance of such wrinkling.

To improve the efficiency of the presently discussed type of paint and varnish remover, I proceeded first with the systematic investigation of the influence exerted by each anti-penetrant separately, i. e., by paraffin wax and by nitrocellulose dissolved in various paint and varnish remover solvents upon the removing action of these solvents. This investigation led to many interesting and important observations which enabled me to produce a combination of ingredients in such a way as to minimize the harmful retarding effect of the above solids in regard to their influence upon cutting speed and efficiency of this type of remover.

The following mixtures of two types of paint and varnish remover solvents, one being a penetrating (or wax solvent) type and the other a loosening (or wax-precipitating) type, were studied, determining first the cutting rate of each mixture without the addition of any solid substance, such as wax or nitrocellulose. This cutting speed will later

be referred to as the "absolute cutting action of a solvent" and is expressed in seconds:

| Solvents                                            | Absolute cutting action—seconds |
|-----------------------------------------------------|---------------------------------|
| Benzol and acetone.....                             | 70                              |
| Benzol and methanol.....                            | 40                              |
| Benzol and methyl acetate.....                      | 45                              |
| Benzol and "lugosol".....                           | 45                              |
| Petroleum naphtha and acetone.....                  | 240                             |
| <b>10</b> Petroleum naphtha and methyl acetate..... | 120                             |

(Petroleum naphtha in these cases had a boiling point range.....60 to 85° C.)

**15** A series of samples were then made with each of the above mixtures incorporating in one case various proportions of paraffin wax; in the second case, various proportions of nitrocellulose (1/2 second viscosity), and in the **20** third case incorporating both wax and nitrocellulose simultaneously. The cutting speed or the activity of each mixture was measured on painted wooden strips as described above and the results obtained were calculated so **25** as to represent a degree of retardation in percent of the absolute removing action of a given solvent combination.

The experiments now to be described show that the influence of paraffin wax and of nitrocellulose upon the activity of a paint and **30** varnish remover is not of the same nature even for a given solvent composition. Examination of the above curves leads to the following conclusions:

**35** Influence of paraffin wax as anti-penetrant:

1. Paraffin wax slowed down the removing action (cutting speed) of paint remover solvent mixtures.

**40** 2. The rate of slowing action or retardation due to the presence of wax, within limits, is proportional to the relative amount of wax included in the remover (roughly).

3. The retardation due to wax is relatively less with petroleum naphtha than with benzol **45** for a given wax precipitant and a given amount of incorporated wax.

Nitrocellulose (1/2 second viscosity) as anti-penetrant:

1. This solid also decreased the removing **50** action or cutting speed of a given solvent combination.

2. The retardation due to nitrocellulose is relatively greater than the retardation due to wax for a given solvent mixture.

**55** 3. For a given solvent mixture retardation due to nitrocellulose is proportional to the amount of nitrocellulose introduced into this solvent (only very roughly).

Anti-penetrants, paraffin wax and nitrocellulose jointly:

1. For a given amount of nitrocellulose and paraffin wax in a given solvent mixture the relative retarding action approximately equals the sum total of individual retardation produced by each substance separately;

for example: For a mixture of various solvents containing 2% of wax and 1% of nitrocellulose (1/2 second viscosity) this retardation was as follows:

|                                           | Found | Calculated | 70 |
|-------------------------------------------|-------|------------|----|
| Benzol and acetone.....                   | 79    | 65         |    |
| Benzol and "lugosol".....                 | 67    | 66         | 75 |
| Benzol and methyl acetate.....            | 44    | 48         |    |
| Benzol and anhydrous methanol.....        | 37    | 38         |    |
| Petroleum naphtha and methyl acetate..... | 48    | 32         |    |
| Petroleum naphtha and acetone.....        | 29    | 29         |    |

In connection with the above figures it should be remembered that they represent only the relative value of the influence of either wax or nitrocellulose upon a combination of two solvents and for practical application they should always be used in reference to the absolute cutting action of a given mixture, as represented in the first table given above. For example: considering two mixtures, (a) benzol and methyl acetate and (b) petroleum naphtha and methyl acetate for a given proportion of nitrocellulose, say 5%, the first mixture will prove more desirable in spite of the greater relative drop in efficiency due to nitrocellulose on account of the higher absolute cutting action of the pure solvent, because the actual activity of each of these removers will be as follows:

For benzol and methyl acetate mixture actual cutting speed will be:

$$70 \text{ seconds} + \frac{70 \times 78}{100} = 70 + 54.6 \quad 100$$

about 124 seconds.

For petroleum naphtha and methyl acetate mixture actual cutting speed will be:

$$240 \text{ seconds} + \frac{240 \times 18}{100} = 240 + 43.4 \quad 105$$

about 283 seconds.

The solvent under the name of "lugosol," mentioned in this specification, is a product obtained from acid-free acetone by treating it with a small amount (a few tenths of one per cent) of caustic alkali, allowing it to condense for a day or more, neutralizing the alkali, and then distilling off unconverted acetone. Such solvent used in above examples was made by adding to one liter of pure acetone one gram of powdered potassium hydroxide. The mixture was allowed to stand at room temperature for about sixty hours, then was neutralized with tartaric acid, the precipitate of potassium tartrate was filtered out and the filtrate was distilled, separating the fraction with the boiling point below 60° C. and the fraction with the boiling point above 60° C. This high boiling fraction represents one form of the solvent called "lugosol." The term "lugosol" is so used throughout the present case.

After determining experimentally the joint 130

retarding action of both anti-penetrants, i. e., paraffin wax and  $\frac{1}{2}$  second viscosity with cellulose for the amount given above, and noting that the experimental data is very close to the volume of retardation calculated from the curves representing the retardation of each individual anti-penetrant, I proceed to determine if such observation will hold true for other variations in the relative amount of each anti-penetrant. The table below shows that this is the case.

*Joint retarding action of*

|                                                  | Found | Calculated |  |
|--------------------------------------------------|-------|------------|--|
| 15                                               |       |            |  |
| 1 per cent nitrocellulose and 1 per cent wax:    |       |            |  |
| Benzol and acetone                               | 55    | 58         |  |
| Benzol and "lugosol"                             | 50    | 50         |  |
| Benzol and methyl acetate                        | 28    | 25         |  |
| Benzol and anhydrous methanol                    | 30    | 25         |  |
| 20 2 per cent nitrocellulose and 4 per cent wax: |       |            |  |
| Benzol and acetone                               | 120   | 127        |  |
| Benzol and "lugosol"                             | 78    | 72         |  |
| Benzol and methyl acetate                        | 60    | 60         |  |
| Benzol and anhydrous methanol                    | 55    | 52         |  |
| 3 per cent nitrocellulose and 3 per cent wax:    |       |            |  |
| Benzol and acetone                               | 100   | 120        |  |
| Benzol and "lugosol"                             | 80    | 76         |  |
| Benzol and methyl acetate                        | 61    | 54         |  |
| Benzol and anhydrous methanol                    | 45    | 43         |  |
| Petroleum naphtha and acetone                    | 35    | 35         |  |

The above figures indicate that the experimentally obtained calculated results can be considered reasonably close in view of the necessarily rather rough character of the tests.

The figures above given show that while one loosening solvent, such as acetone, may be a desirable ingredient in conjunction with one wax solvent, such, for example, as petroleum hydrocarbons, it will not be as suitable in conjunction with other kinds of wax solvents, such as benzol. In this latter case the above data show that if a ketonic solvent is desirable it would be much more advantageous to use "lugosol" than acetone.

In order to confirm these theoretical observations, a number of paint and varnish removers have been made using a series of solvents in accordance with the experimental data above given.

This will be explained in discussing examples given below which illustrate the practical application of the theme of the present invention.

It is understood that all the formulas given below should be regarded only as examples and that I do not wish to restrict myself to the exact components and proportions given in these formulas. The mixtures of solvents in these examples are based on an interpretation of the data given above in such a way as to compose removers from solvents which are less influenced by the addition of wax and nitrocellulose under given conditions, as will be explained in connection with example 9 given below. The cutting speed of each sample was tested on a panel cut from an auto-

mobile body, as already described, and the results of such determination concurred with the assumption drawn from the examination of the above diagrams. In all these examples the amount of solvents, wax and nitrocellulose are given in percent by weight.

*Example 1*

|                                  | Parts |
|----------------------------------|-------|
| Benzol                           | 40    |
| Anhydrous methanol               | 25    |
| "Lugosol"                        | 15    |
| Methyl acetate                   | 15    |
| Paraffin wax                     | 3     |
| Nitrocellulose (scrap celluloid) | 2     |
|                                  | 80    |

The cutting speed of this remover was 80 seconds as against 250 seconds of commercial remover bought on the market and supposed to be one of the most active of the heavy bodied removers on the market. This commercial remover contains benzol as the wax solvent, and the removers in Examples 1 to 5 and about the same "body" (viscosity, flow, etc.) as said commercial remover.

*Example 2*

|                                  | Parts |
|----------------------------------|-------|
| Benzol                           | 40    |
| Anhydrous methanol               | 25    |
| Methyl acetate                   | 30    |
| Paraffin wax                     | 3     |
| Nitrocellulose (scrap celluloid) | 2     |
|                                  | 95    |

The cutting speed of this remover was 65 seconds as against 80 seconds of the remover given in Example 1. It will be noticed that this example differs from Example 1 in the replacement of "lugosol" by methyl acetate. Reference to the above tables shows that benzol and "lugosol" mixture suffers a greater retardation (by adding these amounts of wax and nitrocellulose) than does the benzol, methyl acetate mixture; hence, the conclusion from the diagram would be that if "lugosol" is replaced with methyl acetate the speed of the remover should increase. This observation proved to be correct, as shown by the determination of cutting speed of these two removers.

*Example 3*

|                          |              |
|--------------------------|--------------|
| Benzol                   | 40 parts.    |
| Anhydrous methyl alcohol | 25 parts.    |
| Acetone                  | 15 parts.    |
| Methyl acetate           | 15 parts.    |
| Paraffin wax             | 3 parts.     |
| Celluloid scrap          | 2 parts.     |
| Cutting speed            | 100 seconds. |

The composition of this example differs from the composition given in Example 1 by replacing "lugosol" with acetone.

Reference to the above tables shows that the benzol, acetone mixture suffers a much greater retardation by addition of wax and nitrocellulose, than benzol and "lugosol" mixture, and therefore the replacement of

"lugosol" with acetone would result in the decrease of cutting speed. The comparison of cutting speeds of composition #1 and the present composition concur with that conclusion.

5

*Example 4*

|                                |              |
|--------------------------------|--------------|
| Light petroleum distillate (B. |              |
| P. 60 to 85° C.)               | 30 parts.    |
| Anhydrous methanol             | 25 parts.    |
| 10 Methyl acetate              | 40 parts.    |
| Paraffin wax                   | 3 parts.     |
| Celluloid scrap                | 2 parts.     |
| Cutting speed                  | 240 seconds. |

15

*Example 5*

|                                |              |
|--------------------------------|--------------|
| Petroleum distillate (B. P. 60 |              |
| to 85° C.)                     | 30 parts.    |
| Anhydrous methanol             | 25 parts.    |
| Acetone                        | 40 parts.    |
| 20 Paraffin wax                | 3 parts.     |
| Celluloid scrap                | 2 parts.     |
| Cutting speed                  | 180 seconds. |

In comparing the cutting speeds of Examples #4 and 5, it can be seen that the composition of Example #5 is much speedier than that of Example #4. The difference in the composition of Example #5 is that methyl acetate in Example #4 was replaced 30 with acetone. "Lugosol" could also be substituted.

This increase in speed is in accord with the data showing the petroleum acetone mixture to have a lower retardation than the petroleum methyl acetate mixture.

It is here worthy of remark that although the removers of Examples 4 and 5 both contain petroleum hydrocarbons as wax solvents, 40 both the removers are essentially more highly active than the best heavy bodied removers on the market.

I claim:

1. A finish remover containing petroleum hydrocarbons substantially all boiling at below 85° C., functioning as the essential wax solvent, and containing wax in amount sufficient to give a heavy bodied remover, and containing relatively volatile wax precipitants in such amount as to form a highly active finish remover, the wax precipitants including one at least of the substances of the group consisting of anhydrous methanol, anhydrous methyl acetate, acetone and "lugosol," such remover having a cutting speed of at least 240, the wax precipitants being in excess over the wax solvent.

2. A finish remover having petroleum hydrocarbons consisting wholly of fractions boiling at about 60 to 85° C., as the essential wax solvents, and having sufficiently large proportions of wax and nitrocellulose to produce a heavy body to the remover, and containing wax precipitants in excess of wax solvents, at least the major part of its wax

precipitant selected from the group consisting of substantially anhydrous methanol, methyl acetate, acetone and "lugosol".

3. A finish remover having about the following composition—

|                    | Parts |
|--------------------|-------|
| Benzol             | 40    |
| Anhydrous methanol | 25    |
| "Lugosol"          | 15    |
| Methyl acetate     | 15    |
| Paraffin wax       | 3     |
| Nitrocellulose     | 2     |

4. A finish remover having about the following composition—

|                    | Parts |
|--------------------|-------|
| Benzol             | 40    |
| Anhydrous methanol | 25    |
| Methyl acetate     | 30    |
| Paraffin wax       | 3     |
| Nitrocellulose     | 2     |

5. A finish remover having about the following composition—

|                                                 | Parts |
|-------------------------------------------------|-------|
| Petroleum distillate (B. P. about 60 to 85° C.) | 30    |
| Anhydrous methanol                              | 25    |
| Acetone                                         | 40    |
| Paraffin wax                                    | 3     |
| Celluloid scrap                                 | 2     |

6. A finish remover having the following composition:—

|                                                                                                                                   |                |
|-----------------------------------------------------------------------------------------------------------------------------------|----------------|
| Wax solvent, consisting of hydrocarbons substantially all boiling between about 60 and 85° C.                                     | 30 to 40 parts |
| Wax precipitants selected from the herein described group consisting of anhydrous methanol, methyl acetate, acetone and "lugosol" | 55 to 65 parts |
| Wax and nitrocellulose material together about                                                                                    | 5 parts        |

In testimony whereof I affix my signature.  
BORIS N. LOUGOVOY.

110

115

120

125

130